

## UNITED STATES PATENT OFFICE.

GALE L. ADAMS, OF HUNTINGTON PARK, CALIFORNIA, ASSIGNOR TO STANDARD OIL DEVELOPMENT COMPANY, A CORPORATION OF DELAWARE.

## FLOTATION OIL.

No Drawing. Original application filed January 30, 1924, Serial No. 689,584. Divided and this application filed July 28, 1927. Serial No. 209,189.

The present invention relates to flotation oils such as are used in concentrating ores and is a division of my previous application, Serial No. 689,584, filed January 30, 1924. My invention will be fully understood from the following description.

In flotation processes for concentrating ores, oily materials are agitated with water and ground ore to form a froth or foam which is then separated from the aqueous suspension of gangue. Creosote or pine oil have been used extensively for this purpose, but it is desirable to obtain cheaper substances.

I have found that the residuum from cracking mineral oils, particularly residues from cracking petroleums under pressure, furnishes very desirable flotation material. It is preferable to compound this residuum with other reinforcing materials as, for example, a minor proportion of pine oil, say 15%, but I find that a reinforcing material which is superior to pine oil is had in the residuum from the hydrolysis of sulphated olefins. This latter product is obtained as a by-product in the manufacture of alcohols from olefins where the olefin is absorbed in sulphuric acid under sulphating conditions, as described in U. S. Patents Nos. 1,486,646 granted March 11, 1924, and 1,486,647 granted March 11, 1924. The sulphated olefins are hydrolyzed to form alcohol, dilute sulphuric acid and an oily layer which contains polymerized hydrocarbons and a high percentage of combined sulphur. The chemical nature of this product is not well understood.

In compounding my flotation oil, I prefer to use from 5 to 30% of the polymerized hydrocarbon product, above identified, the balance up to 100% being made up of the residuum from cracking hydrocarbon oils, especially pressure still tars. In some instances a small quantity of an additional frothing agent may be used and I prefer to use a sulphonate derived from the treatment of hydrocarbon oil with concentrated or fuming sulphuric acid, and preparing a sodium or alkaline salt of the sulphuric acid, as will be well understood. The sodium sulphonate may contain about 40% moisture and I ordinarily prefer to employ from 10% to 5% of such sulphonate.

The quantity of flotation oil varies considerably with the character of the ore to be concentrated, but it is generally between the limits of .05 and 1.0%.

As an illustration of the use of my oil, an ore containing 1.9% copper, such as chalcocite and chalcopyrite, is ground and agitated with water in a frothing machine, using 1.4 lbs. of flotation oil per ton of ore. The oil is a compound of 80% pressure still tar, 19.1% residuum from hydrolysis of sulphated olefins, and .9% water-soluble sodium sulphonate derived from petroleum hydrocarbons.

My invention is not to be limited by any theory of the mechanism or activity of my compounds, nor by any example given merely by way of illustration, but only by the attached claims, in which I wish to claim all novelty inherent in my invention.

I claim:

1. A flotation oil which comprises 80% of pressure still tar, slightly over 19% of residuum from hydrolysis of sulfated olefins, and slightly less than 1% of water-soluble sodium sulfonate of petroleum hydrocarbons.

2. A flotation oil which comprises a hydrocarbon residuum from the cracking of petroleum hydrocarbons, a residuum from hydrolysis of sulfated olefins substantially free from sulfonic compounds, and a water-soluble sodium sulfonate of petroleum hydrocarbons.

3. A flotation oil which comprises a hydrocarbon residuum from the cracking of petroleum hydrocarbons, a residuum from hydrolysis of sulfated olefins, and an agent to improve the frothing qualities.

4. A flotation oil which comprises a hydrocarbon residuum from the cracking of mineral oil hydrocarbons, and a residuum from hydrolysis of sulfated olefins.

5. A flotation oil which comprises a hydrocarbon residuum from a cracking of mineral hydrocarbons, and a reinforcing agent.

6. A flotation oil which contains 80% or less of a hydrocarbon residuum from the cracking of mineral hydrocarbons.

GALE L. ADAMS.